

## UNITED STATES PATENT OFFICE

2,225,552

PRODUCTION OF LUBRICANTS FOR  
TEXTILESIvor M. Colbeth, East Orange, N. J., assignor to  
The Baker Castor Oil Company, New York,  
N. Y., a corporation of New JerseyNo Drawing. Application August 31, 1938,  
Serial No. 227,685

6 Claims. (Cl. 252—52)

This invention relates to the production of oil that is particularly useful as a softening agent or lubricant for textile products although its use is not limited to this particular purpose.

5 Heretofore objections and difficulties have been encountered when different sorts of oils have been used as lubricants for textiles. Among the objections that have arisen have been the development of rancidity in the oils or discoloration of 10 the textiles by the oil or both. Some of the oils that have been used for this purpose are difficult to remove, some are quite expensive and some do not possess the desired lubricating properties.

15 Olive oil has heretofore proven to be one of the most satisfactory oils for lubricating textiles as it possesses great lubricating power which enables the fibers that are lubricated with it to slide over each other quite easily, and at the same time its viscosity, specific gravity and iodine value 20 are such as to make it suitable for this purpose.

25 However, olive oil is not entirely satisfactory as a textile lubricant. Some of the objections to it are: it is not colorless as it contains iron and chlorophyl so that there is a tendency to stain the fabric, especially white fabrics; it possesses a noticeable odor that is not pleasing to everyone so that the use is objectionable where the odor is offensive; the source of supply of olive oil is largely in foreign countries and the price thereof 30 varies considerably from time to time; and it contains about 10 to 20 percent of stearin which sometimes crystallizes or hardens in cold weather thus giving rise to the presence of objectionable solid particles in the lubricant which interfere 35 with its smoothness.

Castor oil has also been used as a lubricant for textiles but is not entirely satisfactory for this purpose because it will become rancid due to oxidation that forms by-products such as peroxides.

40 By the present invention a lubricating oil for textiles is economically produced which possesses the desirable lubricating qualities of olive oil without its objectionable properties and is free or substantially free from the presence of impurities 45 that would injure or discolor fabrics or interfere with the lubricating properties of the oil. The lubricating oil for textiles produced by this invention has about the same viscosity, specific gravity and iodine value as olive oil, and at the same time it does not become rancid, it is light in color or practically water white and does not become yellow with age so that it will not stain fabrics, it is free from ingredients that form crystals or hard particles at lowered temperatures, 50 it does not become oxidized at temperatures con-

siderably above room temperature even in the presence of moisture, and it can be cheaply manufactured.

5 In carrying out this invention castor oil is so treated that a product is obtained therefrom which has been found to possess the characteristics mentioned above that make it particularly suitable as a lubricant for textiles without the objectionable features heretofore encountered.

10 The castor oil is so treated that the hydroxy groups therein are first removed therefrom by dehydrating the castor oil until its iodine value is about 140 whereupon the ricinoleic acid radicals therein become linoleic acid radicals. This may be done in the ways already known such, for example, as by treating it with a non-oxidizing mineral acid or other catalyst as mentioned in my application Serial No. 210,428 filed May 27, 1938.

15 After the castor oil has been dehydrated it is hydrogenated to such an extent that the iodine 20 value is reduced to between 80 and 90. This may be accomplished, for example by treating the dehydrated product with hydrogen at a temperature of about 250° C. under pressure. In this way the linoleic acid radicals are changed for the most 25 part to oleic acid radicals, or an isomer thereof, or one of the two double bonds in the molecules of the dehydrated product is saturated. An analysis of the product obtained in this way shows that it is not a mixture made up of molecules 30 having stearic and linoleic acid radicals therein, but is a product obtained by hydrogenating one of the double bonds of the molecules without hydrogenating the other one.

35 This oil or dehydrated hydrogenated product is of a very light color and contains very little if any stearic acid radicals. It does not become yellow with age and can not be easily oxidized so that it does not become rancid. Even if it became oxidized the products of oxidation are stable and free 40 from odor, due to the fact that a hydrocarbon, which is odorless, is split off instead of an aldehyde which has an unpleasant odor.

45 This oil can be satisfactorily used as a lubricant for textiles and is free from the objections encountered in the use of other oils used for this purpose. It can be sulfonated to form water soluble products, or it can be saponified, and the resulting products used for the same purpose, or it can be mixed or emulsified with mineral lubricating oil and used as a textile lubricant. These 50 products do not contain iron or chlorophyl or other coloring materials and can be removed from the textile materials by means of soap or alkaline materials.

5

10

15

20

25

30

35

40

45

50

55

About 85% of castor oil consists of the glyceride of ricinoleic acid which has one double bond and an hydroxyl in its molecule. The dehydrating step appears to remove the hydroxyl and convert the ester into the glyceride of linoleic acid which has two double bonds, and the hydrogenation step appears to saturate one of the two double bonds in each linoleic acid residue in this ester thus converting it into the glyceride of oleic acid or an isomer thereof, with very little if any of the glyceride of saturated acids such as stearic acid or of the glyceride of acids having two double bonds such as linoleic acid therein.

What is claimed is:

- 15 1. A lubricant for textiles and the like comprising dehydrated castor oil having one of the double bonds of each acid group saturated.
2. A lubricant for textiles and the like comprising dehydrated castor oil that has been subjected to about a fifty percent hydrogenation.

3. A lubricant for textiles and the like comprising dehydrated castor oil that has been hydrogenated until its iodine value is between about 80 and about 90.

4. The process of producing a lubricant for textiles and the like which comprises dehydrating castor oil and hydrogenating the dehydrated product until saturation of one of the double bonds of each acid group takes place.

5. The process of producing a lubricant for textiles and the like which comprises dehydrating castor oil and hydrogenating the dehydrated product until it is about half saturated.

6. The process of producing a lubricant for textiles and the like which comprises dehydrating castor oil and hydrogenating the dehydrated product until its iodine value becomes between about 80 and about 90.

IVOR M. COLBETH. 20